

Oct. 16, 1945.

H. W. HOUSTON

2,386,857

POSITIVE REVERSAL PROCESS

Filed April 21, 1943



Fig. 1.



Fig. 2.

INVENTOR  
HERBERT W. HOUSTON  
BY  
HARRIS, KIECH, FOSTER & HARRIS

*Herbert W. Houston*  
FOR THE FIRM

ATTORNEYS.

## UNITED STATES PATENT OFFICE

2,386,857

## POSITIVE REVERSAL PROCESS

Herbert W. Houston, Sherman Oaks, Calif., assignor to The Houston Corporation, Los Angeles, Calif., a corporation of California

Application April 21, 1943, Serial No. 483,916

8 Claims. (Cl. 95—5)

My invention relates to photographic methods, with special reference to film development and is directed specifically to an improved process for producing positive images by reversal.

In prior art practices heretofore prevalent, it has been considered essential to develop the exposed film initially to a relatively high gamma or substantially to completion to preclude any possible existence of a residual latent negative image. Under ordinary and favorable conditions such a process involving initial development to a high gamma results in a final product of acceptable quality, that is to say, the process is satisfactory if the film is given normal or optimum exposure in the camera.

This accepted practice characterized by initial development to a relatively high gamma is not satisfactory over a wide range of exposure. Any degree of over-exposure in the camera causes disproportionate loss in quality in the final positive image, and substantial over-exposure usually results in a completely worthless finished product. The disastrous effect of camera over-exposure in conventional reversal processes may be readily understood when it is considered that the developed negative image is in effect a subtraction from the potential capacity of the film emulsion to provide density in the final positive image. If an excessive proportion of the halide grains in the emulsion is removed, no amount of subsequent exposure of the remaining halide grains will build up an acceptably dense positive image and no photoelectric control system can be operative to compensate for the deficiency.

It is an object of my invention to provide a reversal process effective to produce a positive image of quality over a wide range of departure from normal camera exposure, it being a special object of the invention to extend the range in the direction of over-exposure, thereby to utilize film heretofore regarded as over-exposed beyond retrieve.

Another object of the invention is to provide a reversal process that will produce a higher average quality than heretofore attained when applied to the development of numerous positive reversal films from various sources exposed under diverse circumstances with widely varying degrees of skill. It is proposed to provide a reversal process that may be applied indiscriminately to variously exposed film to provide inherently and automatically compensation for all deviations from normal exposure.

It is a further object of the invention to provide a reversal process which is not critical in

operation and which does not necessitate employment of photo-electric control to meet the varying requirements of variably exposed film.

If the exposed film is initially developed to completion, say, to a gamma of 1.3 to 1.6, the subsequent bleaching operation removes all of the originally activated halide grains. It has heretofore been assumed that any residual activated halide grains comprising the latent negative image will be developed at a later stage in the reversal process to negate the final positive image. One object of my invention is to provide a process that permits incomplete initial development of the potential negative image without involving the usual penalty of subsequently producing a developed residual negative to the material detriment of the final product.

Since initial full development reduces the subsequent image-forming capacity of the film, a film that is over-exposed in the camera and then initially developed to completion in the conventional manner is inherently incapable of producing an adequate positive image. One of the objects of my invention is to achieve an acceptable, if not an excellent, positive image in the case of over-exposed film by making it possible to utilize for the final positive image a substantial portion of the halide grains that are initially activated in the camera as part of the initial latent negative image. I have good reason to believe that in at least one practice of my invention emphasizing the treatment of over-exposed film, at least some halide grains that are initially activated in the camera and survive temporarily as the residual latent negative image are actually deactivated in the course of my process and subsequently respond to light to form density in the final positive image.

A further object of my invention, then, in the practice of my invention that includes processing of over-exposed film is to provide a bleaching agent and a bleaching step that will have the effect of erasing a residual latent negative image, the term "erasing" being used in the sense that the bleach deactivates the grains comprising such residual image and restores the grains to light-responsiveness for subsequent participation in a positive image. In this regard it is also an object of my invention to provide a bleaching agent and a bleaching step that will have, in effect, a certain selective action in the sense that the activated grains comprising the residual latent negative image will be deactivated and yet other co-

existing activated grains of a coexisting latent positive image will survive.

A still further object of my invention is to provide a procedure for developing a positive image involving the use of successive light exposures in such manner as inherently to provide compensation for various degrees of camera exposure of the film.

The above and other objects of my invention will be apparent in the following detailed description, taken with the accompanying drawing.

In the drawing, which is to be regarded as illustrative only:

Fig. 1 is a diagrammatic view largely in section indicating the construction of an apparatus that may be employed in the practice of the invention; and

Fig. 2 is a similar fragmentary view of a modified form of apparatus.

In the simplest practice of my invention the exposed direct positive film is first developed to substantially less than completion and is passed into a stop solution to arrest development. The film is then exposed to the light of a printing lamp with the developed negative image serving as a printing mask. After the printing exposure, the film is passed successively through a bleaching solution and a clearing solution and is then exposed to a second lamp. After the second exposure to printing light, the film is developed, fixed, washed, and dried in the usual manner.

In this procedure the film goes through two cycles of light exposure. In the first cycle, in which the exposure occurs before the bleaching step, a negative image of effective density serves as a mask to favor the printing of a positive image, and in the second cycle, additional grains of silver halide are activated to provide a latent positive image of adequate density. The final development brings out the positive image created by the two printing cycles.

The degree to which initial development is curtailed in the creation of the initial developed negative image will vary in various practices of the invention. Since the purpose of such curtailment is to conserve some of the silver halide grains that are initially light-activated in the camera, the degree of curtailment may be determined in advance more or less precisely in accord with a known need of utilizing in the final positive image a portion of the initially light-activated halide grains. If the degree of over-exposure in the camera is known, such a need may be closely estimated. A feature of the invention, however, is that it is not necessary to ascertain in advance what proportion of the camera-activated grains will be required in a particular instance to avoid deficiency in the final positive image, since curtailment of development of the initial negative image sufficient to take care of a maximum requirement in the positive image will meet all lesser requirements. In other words, a curtailment of the initial negative image development to meet the requirement of a film that is over-exposed in the camera to a given degree will meet the requirements for all films that are over-exposed in the camera to lesser degrees.

Under highly favorable conditions the range of deviation from normal camera exposure may be relatively small, and the need for curtailment of the initial negative image development correspondingly reduced. On the other hand, if the film to be processed covers a wide range of departure from normal exposure, especially in the

direction of over-exposure, rather severe curtailment of initial negative image development will be required. For example, if the process is to be employed for commercial finishing of amateur film from diverse sources or is to be employed to finish film taken under war conditions by the armed services, substantial curtailment will be found desirable. In my preferred practice, curtailment amounts to development of the initial negative image to .65-.75 gamma instead of the usual 1.3-1.6 gamma.

In my preferred procedure, each printing cycle includes development of the film as well as exposure to light, and in each printing cycle a masking image is present on the film. The preferred procedure is as follows. When the initial negative image is developed to substantially less than completion, the film is passed into an acid stop and is then exposed to light from a printing lamp with the negative image serving as a printing mask. After printing exposure, the film passes successively through a bleaching solution and a clearing solution. Preferably the bleaching solution comprises potassium dichromate and sulphuric acid. After the film is bleached and cleared, it is subjected to the action of a developing solution for a period of time sufficient to bring out an initial positive image. With this initial positive image as a mask or shield covering light sensitive halide grains, the film is illuminated by a second lamp, which may be termed a flashing lamp and then the film is again developed. Finally, the film is passed through a stop solution and is fixed, washed, and dried in the usual manner.

It is to be noted that in the described preferred procedure a negative image acts as a printing mask when the film is exposed to the printing lamp and later a positive image acts as a mask when the film is subsequently exposed to the flashing lamp. The masking functions of the two images are quite different from each other. The negative image acts primarily as a reversing mask for determining a pattern of response of halide grains to light. The masking function of the positive image, on the other hand, is not that of reversal but rather is that of retarding or preventing the activation of additional halide grains to increase the density of the positive image, when such increase is not desirable. An important feature of my invention is that the light-restraining effect of the positive image in its function as a mask is automatically and inherently of whatever degree is required by the particular film in view of the degree to which the film has been originally exposed to light in the camera. In other words, the positive image brought out by the initial action of the second developing solution prior to the second exposure to light serves automatically as means to compensate for various degrees of camera exposure and is so effective that automatic printing control by use of photoelectric cells and other expedients is unnecessary.

The curtailment of the first developing step to bring out the negative image at a point substantially short of development to completion necessarily leaves a residual latent negative image represented by a number of light-activated halide grains. Immediately after the development of the negative image is arrested by the initial stop solution, the exposure of the film to the printing lamp with the developed negative image serving as a printing mask results in the activation of a second group of halide grains to

coexist with the first group, the first group comprising the residual latent negative image and the second group comprising the initial latent positive image.

I have discovered that certain bleaching agents may be employed at this stage in my process to result in what seems to be a selective action with respect to the two groups of activated grains, the first group being deactivated to erase the residual latent negative image, and the second group remaining with capacity to form a positive image. Apparently the activated grains comprising the residual latent negative image are not merely deactivated, but are also restored at least to substantial extent to their original state of sensitivity to light.

Bleaching solutions ordinarily used in positive reversal processes do not have such selective and restoring effect on the activated halide grains. Permanganate bleaches, peroxide bleaches, and iodine bleaches, for example, simply destroy both the residual latent negative image and the initial latent positive image. In my preferred practice I employ a dichromate bleach, the proportions being 1% dichromate and  $\frac{1}{2}$  of 1% sulphuric acid in water solution. Dichromate of potassium, dichromate of ammonium, or dichromate of sodium may be used. Another bleach found to be operative in the present process for selective action on the activated halide grains is a copper sulphate iron bleach comprising 1% copper sulphate,  $\frac{1}{2}$  of 1% sulphuric acid, and  $\frac{1}{2}$  of 1% pure iron powder.

I am unable to explain just why my bleach has the selective effect in erasing the residual latent negative image without destroying the latent positive image. At first thought there appears to be no basis on which an explanation of selective action on the two groups of activated grains could be based. On analysis, however, it appears that there may be some basis, first, in the fact that the two groups of grains are activated under different conditions, and, second, in the fact that the two groups of grains are subject to different treatments between the initial activation of the grains and the contact of the grains with the bleach solution. Either of these facts may account for an actual difference in character between the two groups.

With reference to the conditions under which the halide grains are activated, it is apparent that the grains comprising the residual latent negative image are activated in the camera, whereas the grains comprising the latent positive image are activated in the course of processing the film and in the presence of whatever products may be created in the initial developing and initial stopping and may survive to be present when the grains to comprise the latent positive image are activated by the printing lamps. It is conceivable that the two different conditions under which light activation occurs may result in definite distinctions in character of the activated grains.

The possibility of differentiation in character between the two groups of activated grains occurring after initial activation arises from the fact that the activated grains comprising the residual latent negative image are subject to and must survive the initial developing treatment and the initial stop treatment. The grains comprising the latent positive image are activated later and therefore are not subject to such treatments after activation. The treatment may definitely

change the properties of the activated grains of the residual latent negative image.

An alternative explanation for the apparent selective action with respect to the two groups of activated grains is that the effect of the bleach is quantitative rather than qualitative. In other words, it is conceivable that the bleaching agent deactivates and restores grains of both groups simultaneously, but that a substantial or major portion of the activated grains comprising the latent positive image survives after the bleaching action deactivates all of the few grains comprising the residual latent negative image.

Since the initial developed negative image functions as a reversal mask and since the effectiveness of the negative image in blocking light depends upon the degree to which the film is exposed in the camera, I adjust the printing lamps for under-exposed film, that is to say, the first printing lamp is adjusted to match a relatively weak negative masking image. When the light so adjusted is applied to a relatively thin negative masking image, the result is a latent positive image of adequate density. Since, obviously, the density of the initial latent positive image varies inversely as the density of the negative masking image, film that is over-exposed in the camera to yield a strong initial negative image will, when exposed to the first printing lamp, produce a weak and inadequate latent positive image.

When, after exposure to the first printing lamp and treatment by the bleach, a film is immersed in the developing solution the latent positive image develops with a speed that depends upon the strength of the latent positive image. Since a film that is under-exposed in the camera has a strong latent positive image created by the first printing lamp, such a film will in the subsequent developing solution bring out an adequate positive image in a very short period of time. In the practice of my invention in which only two lamps are used, a first printing lamp prior to bleaching and a second flashing lamp after bleaching and initial development, the period of time in which the film is immersed in developing solution immediately prior to exposure to the flashing lamp is sufficient to bring out to adequate density a strong latent positive image on camera under-exposed film. In fact, this initially developed positive image on film that is grossly under-exposed in the camera is such an effective mask that the second cycle of light exposure has little or no effect in activating additional halide grains, and the subsequent or final immersion of the film in the developing solution has substantially no effect other than expected enrichment of the positive image.

Since a weak latent positive image comes out slowly in a developing solution and cannot be given adequate density, even by forced development, film that is over-exposed in the camera and therefore has a relatively weak latent positive image reaches the second light-exposure with a positive image that is too thin to serve as a highly effective mask. The flashing lamp therefore penetrates the initially developed positive image to activate additional halide grains for increase in density of the positive image. Since the film is wet with residual developing solution, additional halide grains turn to silver in the course of exposure to the flashing lamp. If the initially developed positive image needs relatively little increase in density, such increase may occur early in the period of exposure to the flashing lamp, the augmented positive image becom-

ing an effective mask to prevent further increase in halide grain activation. If, on the other hand, the initially developed positive image falls far short of adequate density because the film has been grossly over-exposed in the camera, the whole period of exposure to the flashing lamp may be needed for activation of the required number of additional halide grains. It is apparent that the process automatically compensates for various degrees of camera exposure without the employment of photoelectric control.

In another practice of my invention I add to the preferred procedure described above at least one additional light exposure. The third practice may be carried out as follows. The initial negative image is developed to substantially less than completion in the usual manner, for example, to .65-.75 gamma, whereupon the film is passed into the acid stop. The film is then exposed to the light of a printing lamp with the initial developed negative image serving as a mask. After this first printing exposure, the film is bleached, cleared, and again submerged in a developing solution to bring out an initial positive image, the period of submersion being approximately 25% of the total development time required for a film that is grossly over-exposed in the camera, which film produces a weak initial latent positive image. With this initial positive image serving as a mask, the film is flashed by a lamp and is then developed for approximately 50% of the total development time. Again the film is exposed to a flashing lamp, given the final 25% of development time, and is then fixed and dried in the usual manner.

In this third practice of the invention, a film that is grossly under-exposed in the camera yields a substantially adequate image in the 25% development period and is little affected by the subsequent two flashing lamps. A film that is normally exposed in the camera yields a less effective positive image in the 25% development period and the positive image is brought to a final density in the following 50% development period. A film that is grossly over-exposed in the camera yields a weak and wholly inadequate positive image in the 25% development period, and adequate density is not attained until the last 25% development period. In practice the adjustment of the successive lamps is not critical, it being necessary merely to avoid too drastic exposure in printing the first positive image. Thus the light for printing the initial positive image may, if desired, be so mild that in all instances subsequent light exposure will materially affect the film.

In reviewing the various practices of my invention described above, it is apparent that some of the steps of my process are important for camera under-exposed film, but unimportant for camera over-exposed film, and, conversely, other steps in the process are important for camera over-exposed film and not at all vital for camera under-exposed film. Thus, film that is grossly under-exposed in the camera to produce a relatively thin negative masking image yields a strong initial positive image, the first or printing lamp being of great importance, and the second or flashing lamp being unnecessary. Since, moreover, under-exposure of film in the camera does not seriously deplete the available light sensitive halide grains in the film, it is not essential that the development of the masking negative image be stopped substantially short of completion.

On the other hand, film that is grossly over-exposed in the camera to yield a relatively dense

negative masking image produces a relatively thin initial positive image so that subsequent exposure to the flashing lamp is essential for building up density; also, since camera over-exposure means depletion of light-sensitive halide grains, the stopping of development substantially short of depletion is of utmost importance.

It is apparent, then, that each of the described practices of my invention is the blending of two 10 separate processes, one process being primarily for camera under-exposed film and the other process being primarily for camera over-exposed film. These two processes may be regarded as sub-combinations that may either be brought together as described to make a universal process, or in other practices of my invention may be used as separate processes simplified and specialized for either under-exposed film or over-exposed film.

In considering the various practices of my invention described above, there is good reason to believe that certain additional factors contribute to the success of the process.

One factor arises from the fact that the initial camera exposure of the film to produce the initial 25 latent negative image activates a relatively large proportion of the silver halide grains in the high-light areas of the scene and affects a relatively slight proportion of halide grains in the shadow areas of the scene. Consequently, in the high-light areas there are relatively few halide grains left to respond to light and the few do not include any substantial proportion of highly sensitive halide grains. On the other hand, in the shadow portions of the scene there are relatively 30 great concentrations of halide grains remaining for response to light and these large concentrations include in substantial portion halide grains that are highly sensitive to light. In other words, there is not only a quantitative distinction between the high-light areas and the shadow areas, but also a qualitative distinction, the film having higher speed in the shadow areas. Both of the distinctions, quantitative and qualitative, favor reversal, and even if all of the light-activated grains comprising the latent negative image were removed by development and bleaching, subsequent exposure of the film to light would produce a positive image.

Another factor contributing to favorable differentiation in the speed of various areas of the film is that the products of development are bromides or iodides, which products are agents restraining the responsiveness of the film to light. It is believed that these products of developing 55 the initial masking negative image survive in the areas in which they are produced to favor the creation of the reversed or positive image by reducing the speed of the film in those areas.

It is believed that a further favorable factor 60 may be attributed to the bleaching operation and the particular bleaching agent employed in my preferred practice. It is thought that silver-chromium compounds may be produced in the bleaching operation to survive with restraining effect in the areas of the film which were formerly negative.

Fig. 1 indicates, by way of example, the construction of apparatus that may be employed for carrying out my preferred process in a continuous manner. The exposed direct positive film 10 is led from a reel 11 over a guide roll 12 into an initial developing tank 13, the film in the tank traversing between an upper gang of rolls 15 and a lower gang of rolls 16 for a time period 75 to carry development to approximately .65-.75

gamma. The film with the developed negative image thereon passes over guide rolls 17 and into a tank 18 of stop solution to arrest development. The film is then guided by rolls 19 into the light field of a first printing lamp 20 with the developed negative image serving as a light mask. After this light exposure, the film passes successively through a tank 21 of bleach solution and a tank 22 containing a clearing solution.

The bleached and cleared film passes over guide rollers 23 and makes a number of traverses through a developing solution in a tank 24 sufficient for partial development of an initial positive image. At this juncture the partially developed film is guided by rollers 25 under a second or flashing lamp 26 with the developed or partially developed positive image serving as a mask or shield over the light-sensitive halide grains. After this second printing exposure the film makes sufficient additional traverses in the developing tank 24 for final development of the positive image to adequate density if such final development is required and then passes successively through a tank 27 containing a stop solution, a tank 28 containing a fixing solution, and a wash tank 30. From the wash tank 30 the film is guided by rollers 31 into a suitable drying cabinet generally designated 32, the completely dried film emerging from the cabinet to be wound onto a reel 33.

To carry out the third of the practices described above, the apparatus shown in Fig. 1 may be modified in the manner indicated by Fig. 2. The apparatus shown in Fig. 2 is largely identical to the apparatus shown in Fig. 1, corresponding numerals being employed to designate corresponding parts.

Fig. 2 differs from Fig. 1 in showing a relatively extensive developing tank 35 and in showing, by way of example, two flashing lamps 36 and 37 associated with the final development tank instead of the single printing lamp 26 in Fig. 1. As indicated in Fig. 2, the film passes in the usual manner through the first development tank 13 to develop an initial negative image, and enters the tank 18 to arrest development at a relatively low gamma. The film with the initial negative image serving as a printing mask is then exposed to the first printing lamp 20 and is then carried through the bleach solution in the tank 21 and through the clearing solution in the tank 22. The bleached and cleared film passes over guide rollers 23 and makes a number of traverses through the developing solution in the tank 35 sufficient for partial development of a normal image, which development brings out an initial positive image. The partially developed film is then guided by rollers 25 under the flashing lamp 36. To this point the film has been subjected to the same treatment as in the apparatus shown in Fig. 1, the printing lamp 36 in Fig. 2 corresponding to the printing lamp 26 in Fig. 1.

After printing exposure under the lamp 36, the film again makes several traverses through the developing solution in the tank 35 and is then guided by rollers 40 under the flashing lamp 37, the accumulated image on the film serving as a mask or shield. Again the film makes several traverses through the solution in the tank 35 for final development of the image if such final development is necessary. Finally, the film passes into a stop solution and a fixing solution for finishing in the manner heretofore described.

Since it is difficult to ascertain precisely why my process is successful and so advantageous over prior art procedures I am not to be bound by any explanatory comment herein.

- 5 5 The procedures and apparatus described in detail for the purpose of disclosure and to teach the principles involved will suggest to those skilled in the art various changes and substitutions under my basic concept, and I reserve the right to 10 all departures from my disclosure that properly lie within the scope of my appended claims.

I claim as my invention:

1. A reversal process for exposed film, including the steps of: developing the exposed film to 15 a gamma of approximately one-half that produced by normal development thereof, thereby converting a major portion of the initially light-activated halide grains of the film to form a negative image and leaving unconverted a substantial

20 remaining portion of the initially light-activated halide grains; exposing the film to light with said negative image as a mask to activate additional halide grains in the film; bleaching out the converted grains comprising said developed 25 negative image; again exposing the film to light to activate additional halide grains; developing the film to convert the light-activated grains therein to form a positive image; and fixing the film.

30 2. A reversal process for exposed film, including the steps of: under-developing the exposed film to form a negative image of approximately one-half the gamma produced by normal development thereof; exposing the film to light with

35 said negative image as a mask to activate additional halide grains in the film to form a latent positive image; bleaching out the converted grains comprising said developed negative image; treating the film with a developing agent to bring

40 out at least in part said latent positive image; exposing the film to light with said developed positive image as a mask, thereby activating any additional halide grains in the film necessary to bring said positive image up to adequate density; again treating the film with a developing agent; and fixing the film.

3. A reversal process for exposed film, including the steps of: developing the exposed film to a gamma of approximately one-half that produced by normal development thereof, thereby converting a major portion of the initially light-activated halide grains of the film to form a negative image and leaving unconverted a substantial

55 remaining portion of the initially light-activated halide grains; exposing the film to light with said negative image as a mask to activate additional halide grains in the film to form a latent positive image; bleaching out the converted grains comprising said developed negative image; treating the film with a developing agent to bring

60 out at least in part said latent positive image; exposing the film to light with said developed positive image as a mask, thereby activating any additional halide grains in the film necessary to bring said positive image up to adequate density; again treating the film with a developing agent; and fixing the film.

4. A reversal process for exposed film, including the steps of: developing the exposed film to a gamma of approximately one-half that produced by normal development thereof, thereby converting a major portion of the initially light-activated halide grains of the film to form a negative image and leaving unconverted a substantial remaining portion of the initially light-acti-

vated halide grains; subjecting the film to light exposure with said negative image as a mask to activate additional halide grains in the film for a latent positive image, said exposure being insufficient to result in a positive image of a desired density; bleaching out the converted grains comprising said developed negative image; treating the film with a developing agent to form a positive image; exposing the film to light with said positive image as a mask, thereby activating additional halide grains in the film to compensate for said insufficient exposure; again treating the film with a developing agent; and fixing the film.

5. A reversal process for direct positive film varying in degree from camera under-exposure to camera over-exposure, including the steps of: under-developing the exposed film to a gamma of approximately 0.65, thereby converting a major portion of the initially light-activated halide grains of the film to form a negative image and leaving unconverted a substantial remaining portion of the initially light-activated halide grains; subjecting the film to light exposure with said negative image as a mask to activate additional halide grains in the film for a latent positive image, said exposure being insufficient to create a latent positive image of adequate density in the film areas of extreme camera over-exposure but sufficient for areas of extreme camera under-exposure; bleaching out the converted grains comprising said developed negative image; treating the film with a developing agent to bring out a positive image; subjecting the film again to light exposure with said positive image as a mask, thereby activating additional halide grains in camera over-exposed areas of the film; again treating the film with a developing agent; and fixing the film.

6. A reversal process for grossly over-exposed film, including the steps of: developing the exposed film to a gamma of approximately one-half that produced by normal development thereof, thereby converting a major portion of the initially light-activated halide grains of the film to form a negative image and leaving unconverted a substantial remaining portion of the initially light-activated halide grains; subjecting the film to light exposure with said negative image as a mask to activate additional halide grains in the film for a latent positive image; bleaching out said developed negative image and restoring the light-sensitivity of at least some of said unconverted initially light-activated halide grains; treating the film with a developing agent to bring out an initial positive image of inadequate density; subjecting the film at least once again to light with said initial positive image serving as a

mask, thereby activating additional halide grains; at least once again treating the film with a developing agent; and fixing the film.

7. In a reversal process for exposed film having both camera over-exposed and camera under-exposed scenes thereon, including the steps of: substantially under-developing the film, so that said camera over-exposed scenes are developed to only a relatively low gamma and to form a visible negative image and an invisible latent image of each of said scenes on said film; equally exposing each of said scenes to light and using said visible negative images of each of said scenes as a mask for such exposure, so as to form a relatively weak latent positive image of said camera over-exposed scenes and a relatively strong latent positive image of said camera under-exposed scenes; treating said film with a bleaching agent so as to remove said visible negative image from each of said scenes and so as to resensitize at least a portion of each of said invisible latent images to light; again equally exposing each of said scenes to light so as to strengthen each of said positive images; again developing said film to render visible and of suitable density and gradation all of said positive images; and fixing said film.

8. In a reversal process for exposed film having both camera over-exposed and camera under-exposed scenes thereon, including the steps of: substantially under-developing the film, so that said camera over-exposed scenes are developed to only a relatively low gamma and to form a visible negative image and an invisible latent image of each of said scenes on said film; equally exposing each of said scenes to light and using said visible negative images of each of said scenes as a mask for such exposure, so as to form a relatively weak latent positive image of said camera over-exposed scenes and a relatively strong latent positive image of said camera under-exposed scenes; treating said film with a bleaching agent so as to remove said visible negative image from each of said scenes and so as to resensitize at least a portion of each of said invisible latent images to light; again equally exposing each of said scenes to light so as to strengthen each of said positive images; again developing said film to partially develop and render visible all of said positive images; again equally exposing each of said scenes to light and using said visible positive images as a mask for such exposure, so as to increase the exposure of said positive images in inverse proportion to the density of said visible positive images; again developing said film to increase the density of said visible positive images; and fixing said film.

HERBERT W. HOUSTON.